

Aug. 11, 1925.

W. RAYM

1,549,218

CASTING PROCESS FOR INCORPORATING SHAFTS, JOURNALS, OR THE LIKE

Filed June 6, 1924

Fig. 1.



Fig. 2.



Fig. 3.



Inventor

Willibald Raym,  
By  Atty.

Patented Aug. 11, 1925.

1,549,218

# UNITED STATES PATENT OFFICE.

WILLIBALD RAYM, OF DEUZ, GERMANY.

CASTING PROCESS FOR INCORPORATING SHAFTS, JOURNALS, OR THE LIKE.

Application filed June 6, 1924. Serial No. 718,332.

*To all whom it may concern:*

Be it known that I, WILLIBALD RAYM, a citizen of the German Empire, and resident of Deuz, Westfalen, Germany, have invented certain new and useful Improvements in Casting Processes for Incorporating Shafts, Journals, or the like; and I do hereby declare the following to be a full, clear, and exact description of the invention, such as will enable others skilled in the art to which it appertains to make and use the same, reference being had to the accompanying drawings, and to letters or figures of reference marked thereon, which form a part of this specification.

It is known to incorporate shafts and journals with castings in a direct manner, by casting in order to secure them in same. This, however, is only possible with small castings, since during the contraction of the casting, the incompressibility of the shaft present therein sets up casting stresses which, in the case of large work, either cause the casting to burst at once, or may become dangerous during subsequent use.

The object of the present invention is to provide a process whereby such shafts, journals or other parts can be incorporated direct into even large castings by casting, without any casting stresses being set up in the casting in shrinking. In particular, also, very large rollers, with a cast-in shaft, can be made in this manner.

The process consists in providing a certain free space, corresponding to the shrinkage of the casting around the shaft or the like to be incorporated with the casting. The dimensions of this space are calculated so that, as the casting shrinks it will still exert sufficient pressure on the shaft to hold the same securely in the casting. The space may be produced in various ways, either by surrounding the shaft, at a certain distance, with a tube of thin sheet iron or the like, which will give way under the pressure set up by the contraction; or the intervening space may be filled up with material of any kind, for example a metallic alloy or the like, which melts during the contraction and exudes laterally or is burnt out, or is eliminated in any other way during the contraction.

The accompanying drawing illustrates various methods of carrying out the process and in which—

Figure 1 is a longitudinal section of a roll and its shaft illustrating one way of connecting them.

Fig. 2 is a like view of another way, and Fig. 3 is a cross section illustrating a third mode.

In the embodiment according to Fig. 1 *a* is the shaft to be incorporated by casting, and *b* is the casting, in this case a large roller. In order to allow for the shrinkage of the casting, the shaft *a* is surrounded, prior to the iron being poured round it, with a sheet metal shell *c*, which is held at a certain distance away from the shaft by rings *d* at top and bottom. On the iron being then poured round, in a suitable mould, in the shape of the roller *b*, the tube *c* at first causes a space to be left between the metal and the shaft. As the metal cools, it contracts and gradually presses the tube *c* firmly against the shaft *a*, the air in the intervening space being able to escape above and below. The said space is so calculated that the necessary shrinking on pressure for holding the shaft firmly in the roller can still be exerted. In this way the largest castings can be provided with shafts, journals or other inset parts without any dangerous shrinkage stresses making their appearance during the contraction.

In the embodiment according to Fig. 2, the shaft *a* is surrounded by a metallic alloy *e*, which melts at a lower temperature than the metal of the casting; and as the shrinkage pressure increases, this alloy *e* exudes, above and below, along the shaft *a*, so that, in this case a certain amount of the liquefied alloy, corresponding to the increasing contraction, is expelled.

Instead of a metallic alloy, use may be made of any other substance which melts, burns or vaporizes under the heat of the cast metal.

Fig. 3 represents the cross section of a shaft *a* to be incorporated by casting, which is provided with peripheral grooves *f*. Such grooves may also be provided when a tube surrounding the shaft is used, as in Fig. 1 and also when a metallic alloy or other substance is used, according to Fig. 2. The grooves afford the advantage of facilitating the escape to the air or the exudation of the metallic alloy under the shrinkage pressure. Moreover, in this case, one is not so dependent on the actual temperature of the casting

metal and need not calculate the contraction space so carefully. The surplus alloy then simply runs into the grooves. Finally, the grooves offer the additional advantage of more securely preventing the shaft from turning inside the casting.

By means of this process, the largest castings of any kind can be provided with castings in parts without dangerous casting stresses being produced.

The grooves of the periphery of the shaft may also be arranged in spiral form, and if desired, several sets of such spiral grooves of different pitch can be arranged one above another. Holes, channels or the like may also be provided in the shaft, for the same purpose. Cores, to be subsequently withdrawn from the casting, may also be arranged on the shaft, so that, after providing suitable bores in the shaft, the roller can be cooled from the inside, through the shaft.

I claim:

1. The method of casting about cold, solid cores, which comprises casting a metal about the core in spaced relation thereto, the casting and the core being rigidly connected by the shrinkage of the cast metal.

2. The method of casting about cold solid cores, which comprises surrounding the core with a metal tube, and casting around said tube a metal capable of breaking down the

structure of said tube to provide shrinkage space for the casting.

3. The method of incorporating a cold, solid core with a casting, which comprises separating the core and casting, during the molding of the latter around the core, a distance corresponding to the shrinkage of the casting in cooling.

4. The method of incorporating a cold solid core with a casting, which comprises forming between the core and casting an intervening space of such size as will be taken up by the casting in shrinking.

5. The method of casting about cold solid cores, which comprises forming recesses in the periphery of the core, surrounding the periphery with a tube, and casting around the latter a metal capable of breaking down and forcing the tube into the recesses.

6. The method of casting about cold solid cores, which comprises surrounding the core with a metal tube held in spaced relation from the core, and casting a large body of metal around said tube in contact therewith, said metal operating in shrinking to force the tube into contact with the core.

In testimony that I claim the foregoing as my invention, I have signed my name this 20th day of May 1924.

DPL. INC. WILLIBALD RAYM.